

1

3,336,100

## PROCESS FOR THE PRODUCTION OF MOLYBDENUM DIOXIDE

Raymond Cloppet, La Gifre, France, assignor to Societe d'Electro-Chimie, d'Electro-Metallurgie et des Acieries Electriques d'Ugine, Paris, France, a corporation of France

No Drawing. Filed Feb. 26, 1964, Ser. No. 347,388  
Claims priority, application France, Feb. 28, 1963,  
926,277

6 Claims. (Cl. 23—21)

10

### ABSTRACT OF THE DISCLOSURE

A process for producing molybdenum dioxide by reacting, in stoichiometric amounts,  $\text{MoO}_3$  and  $\text{MoS}_2$  in a temperature range between 600° C. and 700° C. and evolving therefrom free  $\text{SO}_2$  to form a reaction product, and then desulfurizing the reaction product in an atmosphere containing less than 10%  $\text{SO}_2$  at a temperature between 400° C. and 600° C. to obtain molybdenum dioxide, which is then permitted to cool to at least 250° C. in neutral or reducing atmosphere.

This invention relates to preparation of molybdenum dioxide for industrial uses such as production of molybdenum steels and alloys.

Present industrial practices for addition of molybdenum to a bath of liquid steel include placing a quantity of a molybdenum alloy, generally ferromolybdenum, which has the amount of molybdenum required within a solid charge of a furnace before the charge is melted. Another practice comprises adding the ferromolybdenum to the molten bath. Such practices have disadvantages due to the high melting point and great density of ferromolybdenum, which is slow to dissolve in the steel bath because the temperature of the bath is generally lower than the melting point of the ferromolybdenum. Accordingly, the ferromolybdenum remains on the bottom of the furnace and, after tapping out the steel the furnace operator finds pieces of the ferromolybdenum on the bottom of the furnace. Consequently, the steel tapped out is deficient in molybdenum and residual molybdenum left in the furnace is liable to be incorporated into the next heat of steel in which it is unnecessary, or even unwanted, if the next heat requires a low molybdenum content. Thus, consecutive heats of steel may not have the specified amount of molybdenum.

To overcome the foregoing problems, a different practice applies molybdenic oxide,  $\text{MoO}_3$ , which may or may not be accompanied by a reducing agent, onto a steel bath. The reducing action of the iron, and contingently that of the reducing agent, frees the molybdenum which becomes incorporated into the molten bath. However, this method has disadvantages which arise from the molybdenum oxide,  $\text{MoO}_3$ , having a considerable vapor pressure at the temperatures of application. During its loading onto the surface of the liquid steel bath, a substantial proportion is lost by sublimation or by entrainment in the pulverulent condition. In light of the cost of molybdenum, a sizable loss is encountered. Moreover, the amount lost is variable and the steel or alloy may lack the specified amount of molybdenum.

Use of molybdenum dioxide,  $\text{MoO}_2$ , instead of  $\text{MoO}_3$  in this last method of operation offers considerable advantages. In the first place,  $\text{MoO}_2$  requires less reducing agent since it contains no more than 2 atoms of oxygen instead of 3 per atom of molybdenum.

In the second place, it is much less volatile than  $\text{MoO}_3$ , as shown in the following table, wherein percentages rep-

2

resent the molybdenum losses from an identical weight of a solid product heated for 5 minutes within a given current of a gas. To extend testing beyond this period serves no purpose for the reduction of the oxide within the bath of steel occurs very quickly and the loss of molybdenum occurs only before and during this reduction.

| Temperature in ° C. | Loss of Mo in percent of the Mo Present Initially (in the presence of argon or nitrogen) |                |
|---------------------|------------------------------------------------------------------------------------------|----------------|
|                     | $\text{MoO}_3$                                                                           | $\text{MoO}_2$ |
| 800                 | 0.7                                                                                      | 0.2            |
| 1,000               | 23                                                                                       | 2              |
| 1,200               | 86                                                                                       | 8              |

This table thus demonstrates the advantage offered by the dioxide in respect of loss by volatilization.

These advantages must be considered in the preparation of the alloys having a high content of molybdenum, in particular the ferromolybdenum alloys. Such preparation is performed at high temperature by the reduction of molybdenic oxide,  $\text{MoO}_3$ , by an active reducing agent such as aluminum or silicon. Smoke containing a substantial amount of molybdenic oxide which is sublimated is released in abundance during this reaction and the amount of molybdenum in the smoke represents approximately 4% of the weight of molybdenum used in the preparation. The recovery of these dusts requires installation of costly filters which can handle great volumes of gas to be purified within a short time. Such losses of Mo are very greatly reduced by replacing molybdenic oxide with the dioxide,  $\text{MoO}_2$ .

Thus, it is not surprising that the use of  $\text{MoO}_2$  has been recommended for production of molybdenum steel and alloys. However, the different known processes for the production of  $\text{MoO}_2$  by the reduction of  $\text{MoO}_3$  with a gaseous reducing agent such as hydrogen, ammonia or illuminating gas, are too expensive. Also, direct reduction of  $\text{MoO}_3$  by a solid reducing agent such as C or  $\text{MoS}_2$  results in too impure a product which contains residual C or S. In particular, the known processes which react  $\text{MoO}_3$  and  $\text{MoS}_2$  do not include direct preparation of a product having a low sulphur content.

I have found that at a temperature exceeding 400° C., the molybdenum dioxide fixes a quantity of sulphur which increases with the partial pressure of the sulphur dioxide of the atmosphere in which it is generated. The following table shows the sulphur contents of a technical product initially containing S=0.040% which was kept at 650° C. for one-half hour under atmospheric pressure in different atmospheres.

|                         | Percent |
|-------------------------|---------|
| Pure argon              | S=0.020 |
| Argon+10% $\text{SO}_2$ | S=0.081 |
| Argon+30% $\text{SO}_2$ | S=0.134 |
| Argon+50% $\text{SO}_2$ | S=0.165 |
| Pure $\text{SO}_2$      | S=0.215 |

This fixing of sulphur by molybdenum dioxide does not depend only upon the partial pressure of sulphur dioxide, but also upon the length of time of subjection of the dioxide to the particular atmosphere and upon the presence of certain impurities.

My invention relates to a process which includes a reaction of  $\text{MoS}_2$  and  $\text{MoO}_3$  and renders it possible to produce a molybdenum dioxide,  $\text{MoO}_2$ , which has a very low S content and a low  $\text{MoO}_3$  content. Specifically, the process comprises intimately mixing finely divided products containing  $\text{MoO}_3$  and  $\text{MoS}_2$  in stoichiometrical amounts which allow for contingently present impurities liable to react with these two compounds. The resulting mixture is very gradually heated within an enclosure wherein the

atmosphere is conditioned. The reaction between  $\text{MoO}_3$  and  $\text{MoS}_2$  takes place between  $600^\circ \text{C}$ . and  $700^\circ \text{C}$ ., and preferably between  $650^\circ \text{C}$ . and  $700^\circ \text{C}$ ., under a pressure close to and slightly above the atmospheric pressure during which reaction  $\text{SO}_2$  evolves and forms the greater portion of the atmosphere in the furnace until its emission slows down or ceases. Next, the product of the reaction is desulphurized at a temperature exceeding  $400^\circ \text{C}$ ., under a pressure close to atmospheric pressure in an atmosphere poor in  $\text{SO}_2$ , preferably one which contains less than 10%  $\text{SO}_2$ . Finally, the desulphurized product cools to about  $250^\circ \text{C}$ . under a non-oxidizing atmosphere.

The mixture employed in the reaction contains stoichiometrical amounts of oxidizing  $\text{MoO}_3$  and of reducing  $\text{MoS}_2$ . However, my invention is also applicable to constituents which, in addition, contain another oxidizing agent or another reducing agent, and are sources of  $\text{MoO}_3$  or  $\text{MoS}_2$ . The relative quantities of the initial constituents introduced into the reaction enclosures will then be determined, while taking into account the nature and proportion of the oxidizing and/or reducing elements which accompany the  $\text{MoO}_3$  and  $\text{MoS}_2$ . For example, conventional concentrates of molybdenite are not wholly free of the oils used to obtain them by flotation, and this fact should be considered that these oils exert a reducing action upon  $\text{MoO}_3$  in the process. Analogously, if the mixture introduced into the reaction enclosure is the product from a molybdenite roasting kiln, the sulphur it contains must be measured to determine the proportions of the products which are to be mixed in order to practice my process. Moreover, the operation of a roasting kiln of this kind may be regulated so that the product obtained may be used directly in my process.

The physical condition and chemical composition of the products introduced into the kiln or furnace are adapted to the quality of the molybdenum dioxide to be manufactured. In respect to granulometry in particular, it is advisable to use molybdc oxide  $\text{MoO}_3$  whose grains are smaller than 2 mm. The flotation concentrates are appropriate for the  $\text{MoS}_2$ ; however, it is desirable that this  $\text{MoS}_2$  have a high degree of fineness. Additionally, special attention is devoted to stirring of the  $\text{MoO}_3$  and  $\text{MoS}_2$  to obtain an intimate mixture.

The reaction between the  $\text{MoO}_3$  and the  $\text{MoS}_2$  is performed in a hermetic rotary furnace which is equipped with devices for conditioning the atmosphere therein. The reactive mixture is heated progressively and maintained at a temperature exceeding  $650^\circ \text{C}$ . for a certain time, such as several hours. Temperatures which exceed  $700^\circ \text{C}$ . are avoided so as not to effect fritting of the  $\text{MoO}_3$  and  $\text{MoS}_2$ . The time of this heating or first stage depends upon the quality of the product one wishes to obtain, and upon certain characteristics of the reactive mixture, for example, grain sizes, mode of operation, the agitation of the mixture, or the thickness of a solid layer in the furnace.

During this first stage, the atmosphere of the furnace is under pressure in slight excess of that on the outside of the furnace (for instances 5 to 10 mm. of water) and is progressively enriched with  $\text{SO}_2$  until the proportion of  $\text{SO}_2$  exceeds 80%. Naturally, escape of the gases to the outside occurs.

The yield from my process varies according to the operating conditions and may reach 95%.

Generally, this first stage is terminated when the reaction products contain less than 0.5% S and less than 15%  $\text{MoO}_3$ . However, my invention includes commencing the desulphurization, or second stage, earlier and also covers extending the first stage until release of  $\text{SO}_2$  becomes insignificant, i.e. until the pressure inside the furnace stops being superior to the atmospheric pressure, thereby avoiding air entering the furnace.

The residual sulphur content results predominantly from the action of an atmosphere rich in  $\text{SO}_2$  upon the  $\text{MoO}_2$  of the reaction product; half the residual sulphur

results from this action when the  $\text{SO}_2$  content in the atmosphere of the furnace ranges about 80%.

Thus, it is advisable to desulphurize the reaction product, and to achieve same, the product is maintained at a moderately high temperature,  $400^\circ \text{C}$ . to  $600^\circ \text{C}$ ., within an enclosure under a pressure close to atmospheric pressure, in which partial  $\text{SO}_2$  pressure is as low as possible and generally lower than 10%. In this enclosure, the scavenging operation with an inert gas such as nitrogen or argon is one way of effecting the desulphurization. This second stage may be carried out between the end of the reaction and the cooling of the product, or during subsequent reheating of the product after it has been withdrawn from the furnace and after cooling. Very low percentages of S and of  $\text{MoO}_3$  are thus obtained simultaneously in the  $\text{MoO}_2$  product of my process.

If a relatively high content of  $\text{MoO}_3$ , greater than that obtained at the end of the first stage, can be tolerated in the  $\text{MoO}_2$  product while a very low percentage of S is required, the furnace of the second stage is scavenged with a slightly oxidizing current of gas, e.g., one containing a limited quantity of air. The quantity of air —therefore oxygen—to be admitted obviously depends upon the reoxidation of the product which may be tolerated for substantially the whole oxygen so introduced oxides  $\text{MoO}_2$  into  $\text{MoO}_3$ . This lowers the amount of sulphur but increases the content of free  $\text{MoO}_3$  due to a slight reoxidation of the surface of the  $\text{MoO}_2$  product.

In another embodiment of my process, the desulphurization may also be performed at a temperature comprised between  $600^\circ \text{C}$ . and  $700^\circ \text{C}$ . However, one must wait until the emission of  $\text{SO}_2$  has become sufficiently low so that the required rate of flow of the diluent gas necessary for maintaining under 10% the partial  $\text{SO}_2$  pressure in the atmosphere of the furnace is not economically prohibitive. In this embodiment, the reaction between the  $\text{MoO}_3$  and the  $\text{MoS}_2$  may continue to a certain extent with the last traces of reducing sulphur in the reaction product. If in this case the gaseous scavenging necessary to lower the concentration of sulphur dioxide is performed with air, the resulting oxidation on the surface of the molybdenum dioxide may even hasten the end of the reaction. Accordingly, very low sulphur contents are attained in the  $\text{MoO}_2$  product, and the termination of the reaction limits the increase in the content of free  $\text{MoO}_3$  in the  $\text{MoO}_2$  product in comparison with that attained by scavenging with a slightly oxidizing gas at less than  $600^\circ \text{C}$ .

The cooling of the product rich in  $\text{MoO}_2$  is carried out in a non-oxidizing atmosphere, neutral or reducing, to about  $250^\circ \text{C}$ ., to prevent its reoxidation. The inert atmosphere employed for the desulphurization stage is particularly suitable.

In one application of my process, the second stage, desulphurization, occurs in the same furnace as the first stage, wherein the atmosphere is modified so that it contains less than 10%  $\text{SO}_2$ .

In another embodiment of my process, the reaction products are withdrawn from the furnace at the end of the first stage and introduced into another enclosure in which are conditions favorable for desulphurization.

Also, the process may be conducted continuously from the mixing to the extraction of the final cooled  $\text{MoO}_2$  product. It is further possible to practice the process by forming within an identical apparatus two enclosures separated by a partition wherein the lower extremity is immersed in the product which is being processed.

The following are non-limiting examples of my process.

#### Example I

100 kg. of molybdc oxide of technical quality, containing 92%  $\text{MoO}_3$ , and 14 kg. of molybdenite concentrate containing 86%  $\text{MoS}_2$ , were carefully mixed and then treated in a rotary furnace in which they progressively reached a temperature of  $650^\circ \text{C}$ . In this furnace, they

were maintained at this temperature for approximately 3 hours under a pressure close to atmospheric pressure. The furnace was equipped with devices for temperature control and atmosphere conditioning. When the atmosphere in the furnace contained 80% of  $\text{SO}_2$ , the release of sulphur dioxide had practically stopped. Thereafter, the temperature of the furnace was allowed to drop to 500° C. and the atmosphere in the furnace was diluted with a current of nitrogen in such manner that the concentration of sulphur dioxide was kept below 10%. At the end of an hour, heating was stopped, and the inert atmosphere maintained above the product until the temperature dropped to 200° C. The product withdrawn contained:

|                  | Percent | 15   |
|------------------|---------|------|
| S                |         | 0.10 |
| MoO <sub>3</sub> |         | 5.20 |

*Example II*

100 kg. of technical molybdenic oxide and 15 kg. of 20 molybdenite concentrate were intimately mixed and introduced continuously into a rotary furnace equipped with devices for atmosphere control. After a progressive rise in temperature, the mixture remained for approximately 2 hours at a temperature maintained between 25 600° C. and 650° C. The atmosphere of the furnace attained a sulphur dioxide content of 80%. Subsequently, the product was cooled and emerged from the furnace at a temperature of 200° C. It contained:

|                  | Percent | 30   |
|------------------|---------|------|
| S                |         | 0.34 |
| MoO <sub>3</sub> |         | 6.10 |

This product was then introduced into a second furnace substantially identical with the first and equipped with devices for the conditioning of the atmosphere. There it remained for approximately 2 hours at 600/650° C. while subjected to an atmosphere whose sulphur dioxide content was maintained at 10% by blowing in approximately 2 m.<sup>3</sup> of air per 100 kg. of product. The resultant product removed from the furnace at a lower temperature than 200° C. contained:

|                  | Percent | 35    |
|------------------|---------|-------|
| S                |         | 0.080 |
| MoO <sub>3</sub> |         | 7.60  |

*Example III*

In this example, I employed an oxide direct from roasting of molybdenite concentrates within a specially controlled furnace. The oxide contained:

|                   | Percent | 40 |
|-------------------|---------|----|
| MoO <sub>2</sub>  |         | 42 |
| MoO <sub>3</sub>  |         | 48 |
| MoS <sub>2</sub>  |         | 2  |
| Insert substances |         | 8  |

This oxide was mixed with 9 kg. of molybdenite concen-

trate and treated as in Example I. At the end of the operation, a product was obtained containing:

|                  | Percent | 6    |
|------------------|---------|------|
| S                |         | 0.10 |
| MoO <sub>3</sub> |         | 6    |

While I have shown and described preferred embodiments of my invention, it may be otherwise embodied within the scope of the appended claims.

I claim:

1. A process for the production of molybdenum dioxide comprising:
  - (A) mixing finely divided products containing stoichiometric amounts of MoO<sub>3</sub> and MoS<sub>2</sub> to form a reaction mixture;
  - (B) heating said reaction mixture to substantially between 600° C. and 700° C. in a closed chamber to freely evolve SO<sub>2</sub> and maintaining a pressure in the chamber slightly above atmospheric pressure to prevent air from entering the chamber thereby forming a reaction product having a low sulfur content;
  - (C) desulphurizing said reaction product in an atmosphere that contains less than 10% SO<sub>2</sub> and at a temperature substantially between 400° C. and 600° C. to obtain molybdenum dioxide; and
  - (D) cooling said molybdenum dioxide to at least 250° C. under one of a neutral and of a reducing atmosphere.
2. The process of claim 1 characterized by said MoO<sub>3</sub> being grains smaller than 2 mm.
3. The process of claim 1 characterized by carrying out said heating and maintaining until the atmosphere of a furnace in which said heating and maintaining is performed is more than 80% SO<sub>2</sub>.
4. The process of claim 1 characterized by carrying out said heating and maintaining until the sulphur content of the reaction product is less than 0.5% sulphur and less than 15% MoO<sub>3</sub>.
5. The process of claim 1 characterized by during said desulphurizing subjecting said reaction product to flows of an inert gas to maintain the SO<sub>2</sub> content of said atmosphere less than 10%.
6. The process of claim 1 characterized by during said desulphurizing subjecting said reaction product to a gas less oxidizing than air.

**References Cited**

**UNITED STATES PATENTS**

|    |           |         |                 |         |
|----|-----------|---------|-----------------|---------|
| 50 | 1,637,838 | 8/1927  | Simonds         | 75—6    |
|    | 2,398,114 | 4/1946  | Rennie          | 23—21 X |
|    | 2,817,583 | 12/1957 | Schlecht et al. | 75—7    |
|    | 2,987,392 | 6/1961  | Supiro          | 75—90   |

55 OSCAR R. VERTIZ, *Primary Examiner.*

H. T. CARTER, *Assistant Examiner.*